# EUROPEAN PATENT SPECIFICATION

(11) **EP 0 996 545 B1**
(45) Date of publication and mention of the grant of the patent: **18.12.2002**
(21) Application number: 97931905.0
(22) Date of filing: 11.07.1997
(51) Int. Cl.: B41C 1/14

(54) **SCREEN PRINTING STENCIL PRODUCTION**
HERSTELLUNG EINER SIEBDRUCKSCHABLONE
PRODUCTION DE STENCIL SERIGRAPHIQUE

(43) Date of publication of application: 03.05.2000
(73) Proprietor: AUTOTYPE INTERNATIONAL LIMITED, Wantage Oxfordshire OX12 7BZ (GB)
(72) Inventor: FOSTER, David, Joseph, Wiltshire SN1 4NQ (GB); HARRIS, Anna, Jane, Oxfordshire OX12 9DX (GB)
(74) Representative: W.P. THOMPSON & CO.
(86) International application number: GB9701881
(87) International publication number: WO99002344

(56) References cited:
- EP-A- 0 108 509
- EP-A- 0 710 552
- US-A- 5 188 664

## Description

The present invention relates to the production of stencils for screen printing.

### Related Background Art

The production of screen printing stencils is generally well known to those skilled in the art.

One method, referred to as the "direct method" of producing screen printing stencils involves the coating of a liquid light-sensitive emulsion directly onto a screen mesh. After drying, the entire screen is exposed to actinic light through a film positive held in contact with the coated mesh in a vacuum frame. The black portions of the positive do not allow light to penetrate to the emulsion which remains soft in those areas. In the areas which are exposed to light, the emulsion hardens and becomes insoluble, so that, after washing out with a suitable solvent, the unexposed areas allow ink to pass through onto a substrate surface during a subsequent printing process.

Another method, referred to as the "direct/indirect method" involves contacting a film, consisting of a pre-coated unsensitised emulsion on a base support, with the screen mesh by placing the screen on top of the flat film. A sensitised emulsion is then forced across the mesh from the opposite side, thus laminating the film to the screen and at the same time sensitising its emulsion. After drying, the base support is peeled off and the screen is then processed and used in the same way as in the direct method.

In the "indirect method" a film base is pre-coated with a pre-sensitised emulsion. The film is exposed to actinic light through a positive held in contact with the coated film. After chemical hardening of the exposed emulsion, the unexposed emulsion is washed away. The stencil produced is then mounted on the screen mesh and used for printing as described above for the direct method.

In the "capillary direct method" a pre-coated and pre-sensitised film base is adhered to one surface of the mesh by the capillary action of water applied to the opposite surface of the mesh. After drying, the film is peeled off and the screen then processed and used as described for the direct method.

In addition to the above methods, hand-cut stencils can be used. These are produced by cutting the required stencil design into an emulsion coating on a film base support. The cut areas are removed from the base before the film is applied to the mesh. The emulsion is then softened to cause it to adhere to the mesh. After drying, the base is peeled off. The screen is then ready for printing. This method is suitable only for simple work.

One problem generally associated with all the prior art methods is that many steps are necessary to produce the screen, thus making screen production time-consuming and labour-intensive.

Another problem is that normal lighting cannot be used throughout the screen production process in any of the methods except hand cutting. This is because the stencil materials are light-sensitive. In addition, it is necessary to provide a source of actinic (usually UV) light for exposing the stencil. This usually incurs a penalty of initial cost, space utilisation and ongoing maintenance costs.

Other methods of preparing printing screens are available. CA-A-2088400 (Gerber Scientific Products, Inc.) describes a method and apparatus in which a blocking composition is ejected directly onto the screen mesh surface in a pre-programmed manner in accordance with data representative of the desired image. The blocking composition directly occludes areas of the screen mesh to define the desired stencil pattern.

EP-A-0492351 (Gerber Scientific Products, Inc.) describes a method where an unexposed light-sensitive emulsion layer is applied to a screen mesh surface and a graphic is directly ink-jet printed on the emulsion layer by means of a printing mechanism to provide a mask through which the emulsion is exposed before the screen is further processed.

Both the above methods require the use of very specialised equipment (because of the need to handle large complete screens) which incurs a certain cost as well as imposing restrictions arising from the limitations of the equipment, in particular in terms of the size of screen and its resolution.

Ink-jet printers operate by ejecting ink onto a receiving substrate in controlled patterns of closely spaced ink droplets. By selectively regulating the pattern of ink droplets, ink-jet printers can be used to produce a wide variety of printed materials, including text, graphics and images on a wide range of substrates. In many ink-jet printing systems, ink is printed directly onto the surface of the final receiving substrate. An ink-jet printing system where an image is printed on an intermediate image transfer surface and subsequently transferred to the final receiving substrate is disclosed in US-A-4538156 (AT&T Teletype Corp.). Furthermore, US-A-5380769 (Tektronix Inc.) describes reactive ink compositions containing at least two reactive components, a base ink component and a curing component, that are applied to a receiving substrate separately. The base ink component is preferably applied to the receiving substrate using ink-jet printing techniques and, upon exposure of the base ink component to the curing component, a durable, crosslinked ink is produced. US-A-5188664 (Hewlett-Packard) discloses ink compositions for ink-jet use containing 0.2 wt % borox.

### SUMMARY OF THE INVENTION

According to the present invention there is provided a method of producing a screen-printing stencil having open areas and blocked areas for respectively passage and blocking of a printing medium, the method comprising:
providing a receptor element comprising an optional support base and an image-receiving layer capable of receiving a first chemical agent in areas corresponding to the blocked areas of the stencil to be produced;
applying the first chemical agent to the image-receiving layer of the receptor element in the said corresponding areas;
applying a second, stencil-forming chemical agent to a screen printing screen;
bringing the image-receiving layer of the receptor element into contact with the stencil-forming agent, to allow the first and second chemical agents to react to produce on the screen a stencil-forming layer having areas of lower solubility corresponding to the said blocked areas and areas of higher solubility in areas corresponding to the open stencil areas;
removing any remaining unreacted part of the receptor element; and
washing away the second chemical agent in the higher solubility areas, thereby to produce the screen-printing stencil.

In the method of the invention, the stencil is formed by chemical means without the need to use either special lighting conditions or actinic radiation.

Also, it is possible to carry out the. method at reduced expenditure of time and labour, compared with the known processes.

The steps of removing any remaining unreacted part of the receptor element and of washing away the second chemical agent in the higher solubility areas can be carried out in either order or simultaneously. Thus, when the unreacted part of the receptor element comprises a coherent film (for example the optional support base referred to or the image-receiving layer itself), the film can be removed, for example by being peeled away, before the washing away step. Alternatively, the film can be removed in the course of the washing away step, either by the washing action or otherwise, or even be removed after the washing away step. In some cases however the remaining unreacted part of the receptor element may be a material which is removed by the washing action, for example when the optional support base is absent and the image-receiving layer is insufficiently coherent to be removed as an intact layer, for example by peeling away.

Advantageously, the first chemical agent is applied dropwise to the image-receiving layer.

Conveniently, the dropwise application is by use of an ink-jet device, for example an ink-jet printer or plotter. The device may have one or more ejection heads.

If desired, the first chemical agent may be produced in situ by reaction between two or more precursor materials, separately applied to the image-receiving layer, prior to contact with the stencil forming agent, at least one of which is applied in the said areas corresponding to the blocked areas of the stencil to be produced. This may conveniently be achieved by use of a plurality of drop-ejection heads.

When dropwise application is employed, the application is preferably controlled according to data encoding the desired pattern of blocked and open areas of the stencil to be produced. This control is conveniently by a computer, for example a personal computer. Thus, data representative of the desired output pattern can be input to a controller as prerecorded digital signals which are used by the ejection head to deposit or not deposit the liquid containing the chemical agent as it scans the surface of the receptor element. The invention is not however restricted to dropwise application of the first chemical agent: other methods of application will achieve the same essential end, for example, the first chemical agent could be applied with a hand-held marker pen.

The method according to the invention can be carried out using a material of the image-receiving layer which is essentially unreactive with the first chemical agent. In such a process, the image-receiving layer acts essentially as an inert carrier for the first chemical agent. The stencil-forming layer of the eventual stencil is thus derived essentially from the second chemical agent applied to the screen.

Preferably however the material of the image-receiving layer is selected to react with the first chemical agent to produce lower solubility areas corresponding to the said blocked areas and excess of the first chemical agent (or a component of it, not necessarily the same as the component that reacts with the image-receiving layer) remains in said areas to react with the second chemical agent upon contact between the image-receiving layer and the stencil-forming agent, whereby the respective lower solubility areas of the image-receiving layer and of the stencil-forming layer combine with one another and, after the higher solubility areas are washed away, remain to form the blocked areas of the screen-printing stencil.

In such a method, the stencil-forming layer of the eventual stencil is derived in part from the second chemical agent and in part from the image-receiving layer of the receptor element. In this case, the thickness of the stencil-forming layer can be such as to give the eventual screen a "profile", that is a significant thickness to the closed areas of the stencil beyond the thickness of the screen itself. This is of benefit in terms of the quality of printed images which are obtainable by use of the screen as it allows a significant ink deposit to be applied during printing and permits more precise control of the amount of ink deposited. It also produces a flat printing surface which gives better resolution and improved definition by limiting ink spread during printing.

In one variant of the method of the invention, the second chemical agent is applied to the screen printing screen from one side thereof after the receptor element has been applied to the other side thereof with its image-receiving layer in contact with the screen, whereby the image-receiving layer is brought into contact with the second chemical agent.

In another variant, the second chemical agent is applied to the screen printing screen and the receptor element is subsequently brought into contact with the screen to bring the image-receiving layer thereof into contact with the second chemical agent.

### DETAILED DESCRIPTION OF THE INVENTION

The invention will be described further by way of example with reference to the drawings of this specification, in which
Figures 1 to 5 show schematically the successive steps in the production of a printing screen in accordance with one method according to the invention, and
Figures 6 to 10 show schematically the successive steps in the production of a screen in accordance with a second method according to the invention.

Referring to Figures 1 to 5, these show the formation of a screen printing stencil shown in Figure 5, starting with a receptor element shown in Figure 1.

Figure 1 shows the receptor element which consists of an image-receiving layer 1 coated on a flexible film support base 2. In this example, the image-receiving layer is about 10 µm in thickness and the support base about 75 µm.

Figure 2 shows a first chemical agent 3 being applied to the image-receiving layer 1 in droplets 3 which are ejected from an ejection head (not shown) of, for example, an ink-jet printer controlled by a computer. The first-chemical agent 3 is absorbed into the image-receiving layer 1 to form areas 4 which correspond to the blocked areas of the stencil to be formed.

Figure 3 of the drawings shows a screen mesh 5 to one surface of which the receptor element of figure 2 has been applied and to the other of which a stencil-forming agent 6 is being applied using a suitable spreader 7. In figure 3 the image-receiving layer 1 of the receptor element is brought into contact with the stencil-forming agent 6 when the latter is forced through the mesh 5 by the spreader 7.

This contact could alternatively have been achieved by first coating the mesh 5 with the stencil-forming agent 6 and then applying the receptor element to the mesh 5.

Figure 4 of the drawings shows the receptor element 1 consisting of the support base 2 and the image-receiving layer 1, including the areas 4 where the first chemical agent was absorbed, being peeled away from the screen mesh 5. The areas of the stencil-forming agent 6 corresponding to the areas 4 of the image-receiving layer have reacted with the first chemical agent to produce areas 8 of insoluble material'.

Figure 5 shows the final screen after the support base 2 has been peeled away and the screen washed out so that the reduced-solubility areas of the stencil-forming agent in the areas 4 of the image-receiving layer to which the first chemical agent was applied remain and the higher solubility areas have been washed away.

Figures 6 to 10 of the drawings correspond to figures 1 to 5 but show the production of a stencil using a receptor element having an image-receiving layer which reacts with the first chemical agent to produce areas which become incorporated into the stencil-forming layer of the final stencil.

Reference numerals increased by "10" are used in figures 6 to 10 to identify integers corresponding to integers of figures 1 to 5.

Figures 6 to 8 show operations corresponding to the operations of figures 1 to 3. In figure 7 the first chemical agent 13 reacts with the image-receiving layer 11 in the areas 14 but excess of the first chemical agent remains in those areas, to react with the stencil-forming agent 16 as it is applied as shown in figure 8.

Figure 9 therefore shows that, as the support base 12 is peeled away, the areas 14 of the image-receiving layer have become combined with the areas 18 of the stencil-forming layer. and, as shown in figure 10 after washing out, remain in the final stencil to provide the desirable "profile" to which reference has already been made. The remaining, unreacted areas of the image-receiving layer are washed away with the high solubility areas 16 of the stencil-forming layer in the subsequent washing step.

When the image-receiving layer is substantially inert to the first chemical agent it can comprise an inert polymer such as methyl hydroxy propyl cellulose which is preferably present in the image-receiving layer in an amount of 5 to 100 wt.% with the balance comprising, for example, suitable other polymers and/or suitable fillers, binders and plasticisers.

Numerous other inert polymers could alternatively be utilised in the present invention. Suitable polymers include those that have no chemical reaction or only an insignificantly slow chemical reaction with the first chemical agent to be used. Examples of such polymers are:
carboxymethyl cellulose;
polyvinylpyrrolidone; and
polyacrylic acids.

In addition, papers, including ordinary papers, can be used as the inert image-receiving layer, and, thereby, require no supporting base.

The key criterium in selecting a suitable combination of image-receiving layer and first chemical agent is that the first chemical agent should form a good image on the layer; for example, a drop of the first chemical agent should neither be so repelled by the layer as to produce a defective image nor it should not spread so far as to reduce the resolution of the image. Moreover, it should not spread so anisotropically (because of irregularities in the layer) as to deform the image.

When the image-receiving layer reacts with the first chemical agent and thus forms a part of the final screen stencil, the image-receiving layer may comprise a polymer which reacts with the first chemical agent. When the stencil-forming agent is applied and reacts with the first chemical agent (or a component of it, not necessarily the same as the component that reacts with the image-receiving layer), the layer of stencil-forming agent and the reacted part of the image-receiving layer become essentially one.

A typical example of such a polymer is polyvinyl alcohol which is preferably present in an amount of 5 to 100 wt.% of the image-receiving layer with the balance comprising, for example, other suitable polymers and/or suitable fillers, binders and plasticisers. The polyvinyl alcohol preferably has a degree of hydrolysis of 20 to 99.9 mole % and, independently thereof, a degree of polymerisation of 100 to 3500.

Numerous other reactive polymers could alternatively be utilised in the present invention. Suitable polymers include those that change their solubility characteristics on treatment with a suitable first chemical agent. Examples of such polymers are:
gelatin and its derivatives;
carboxylated polymers capable of becoming water soluble on addition of alkali, including carboxylated acrylics, ethylene-acrylic acid and styrene-acrylic acid copolymers;
cellulose derivatives that are water soluble, including starch and hydroxypropyl cellulose;
sulphonated polymers;
polyacrylamides;
epoxy resins; and
amino resins, including urea-formaldehyde and melamine-formaldehyde.

In methods of either type according to the invention, the polymers and other components are chosen so that the first chemical agent forms a good image when applied. Layers that are not compatible with any solvent used in the first chemical agent (typically, water) will produce insufficient spread of the liquid and a poor-quality image will result. If the layer has too great an affinity with the first chemical agent, the liquid will spread too far, giving a blurred, low resolution image.

A receptor element can be with or without a support base. Without the support base, the image receiving layer is typically 6 to 250 µm in thickness. With a support base the coating thickness is typically from 0.1 to 50 µm.

The support base may comprise a non-reactive polymer, preferably an organic resin support, e.g. polyethylene terephthalate, polyethylene, polycarbonate, polyvinyl chloride or polystyrene. Alternatively a coated paper could be used as the receptor element, the paper and coating constituting the support base and the image-receiving layers, respectively. An uncoated paper can alternatively constitute the image-receiving layer of a receptor element without a support base. Such an image-receiving layer is usually removed as a coherent film prior to washing away of the high solubility areas of the stencil-forming layer. The thickness of the support base film is preferably from 10 to 200 µm. The organic resin supports can optionally be coated with a subbing layer to give desired adhesion properties with the image-receiving layer. When used, the support base is usually removed as a coherent film in the screen production method prior to the removal of the areas of higher solubility, though it can be removed during this process.

The first chemical agent is applied to the image-receiving layer. The liquid may be applied dropwise, conveniently by an ink-jet system such as (but not confined to) an ink-jet printer or ink-jet plotter. Alternatively, application can be continuous, for example by a hand held delivery device, such as a pen. The liquid applied should exhibit desirable stability, surface tension and viscosity characteristics and may therefore contain surfactants, viscosity modifiers, light stabilisers and/or anti-oxidants. When the active component(s) of the first chemical agent is/are not liquids, the first chemical agent may include a suitable carrier, for example a suitable solvent or dispersant for the active component(s). The first chemical agent preferably constitutes from 0.5 to 100 wt.% of the first chemical agent.

Examples of suitable active components include boron salts e.g. boric acid, Group I and Group II metal borates; aldehydes, e.g. formaldehyde;
dialdehydes, e.g. glyoxal and glutaraldehyde, optionally activated by treatment with mineral acid;
isocyanates and their derivatives, e.g. toluenediisocyanate; carbodiimides and their derivatives, e.g. 1,3-dicyclohexylcarbodiimide;
transition metal compounds and complexes, e.g. pentahydroxy(tetradecanoate)dichromium and its derivatives; aziridine and its derivatives;
amines;
multifunctional silane compounds, e.g. silicon tetraacetate; N-methylol compounds, e.g. dimethylolurea and methyloldimethylhydantoin; and
active vinyl compounds, e.g. 1,3,5-triacryloyl-hexahydro-s-triazine.

For use in a dropwise application device such as an ink-jet printer or plotter the invention provides a pre-filled cartridge for such a device, the cartridge containing a chemical agent which comprises one or more of the above as an active component in an amount of from 0.5 to 100 wt % optionally in a suitable liquid solvent or carrier.

In the method of the invention the receptor element having had the first chemical agent applied to it may be placed on a solid flat surface and a screen mesh is placed on top such that there is close contact between the mesh and the receptor element. The stencil-forming agent is then typically applied to the screen mesh by a coating trough or squeegee whereby the first chemical agent is brought into contact with the stencil-forming agent, and reacts therewith so reducing its solubility in predetermined areas. Alternatively, a thin layer of the stencil-forming agent can be coated onto the screen mesh, for example by a coating trough or squeegee and the receptor element mounted manually with slight pressure, a technique well-known to those skilled in the screen printing art.

A typical example of a stencil-forming agent comprises an aqueous solution, dispersion or emulsion of polyvinyl alcohol, with a degree of hydrolysis of 20 to 99.9 mole % and a degree of polymerisation of 100 to 3500, as the reactive polymer in proportion of 5 to 100 wt.% and the remainder of the layer contains polymers, fillers, binders and plasticisers as normally found in the art.

Numerous other active polymers could alternatively be utilised as stencil-forming agents in the present invention. Examples of such polymers are:
gelatin and its derivatives;
carboxylated polymers capable of becoming water soluble on addition of alkali, including carboxylated acrylics, ethylene-acrylic acid and styrene-acrylic acid copolymers;
cellulose derivatives that are water soluble, including starch and hydroxypropyl cellulose;
sulphonated polymers;
polyacrylamides;
epoxy resins; and
amino resins, including urea-formaldehyde and melamine-formaldehyde.

If a support base is used, this can conveniently be removed once the reaction of the first chemical agent with the stencil-forming agent has substantially been completed. The resulting screen stencil can be developed by washing away the portion of higher solubility with a suitable solvent, thereby leaving behind areas of reduced solubility to occlude areas of the mesh (this act of washing could also remove the optional support base and any other coherent film part of the receptor element if not removed earlier).

Optionally, the stencil can be further toughened by a post-treatment, for example using extra chemicals, actinic radiation or heat. The extra chemicals (or precursors thereof) may be resident in the original image-receiving layer or in the stencil forming agent, or may be supplied externally. Examples of chemical toughening agents are ones operating at pH 7 or higher and include dialdehydes particularly glyoxal, and aqueous bases, for example aqueous potassium carbonate. It is presently believed that these toughening agents will only work when a boron salt is used as the first chemical agent.

The screen produced is then ready for use as a printing medium using techniques familiar to those skilled in the art. Where the chemicals used are those cited in the Examples 1 to 8 which follow, the broad physical properties, chemical resistances, washout solvent (water) and reclaim chemicals (typically periodate systems) will in many cases be those used routinely by screen printers. So, although the method of producing the stencil is new, the resulting product will often be familiar and highly acceptable to screen printers.

Surprisingly, we have found that when the active component of the first chemical agent is a boron-containing salt, the stencil can be reclaimed with dilute acid without the use of the industry-standard periodate system. This low cost and environmentally-friendlier reclaim system is a distinct added advantage.

The advantages of the method of the present invention include: a screen stencil can be produced directly from digital information sources; unlike the methods disclosed in CA-A-2088400 and EP-A-0492351 which ink-jet print onto a screen mounted in a frame, it is possible to use any general-purpose ink-jet printer using rolls or sheets of film; it is not necessary to use safe-lights during the stencil making process; there is no requirement for an exposure step utilising an actinic radiation source; and a finished stencil can be produced in a shorter time than by conventional screen printing techniques.

The present invention is illustrated by the following examples without however being limited thereto. In these examples, various commercially-available materials are listed by their trade names; the following letters identifying the following companies:
(a) 3M, UK
(b) Autotype International, UK
(c) DuPont, UK
(d) Nippon Gohsei, Japan
Examples 1 to 4 involve the use of non-reactive image-receiving layers; examples 5 to 8 involve the use of reactive image-receiving layers.

### EXAMPLE 1

A liquid containing a first chemical agent was prepared according to the formula:
water - 87 wt.%;
potassium tetraborate - 10 wt.%;
borax - 2 wt.%; and
"Fluorad FC-93" (a) (1wt. % aqueous solution) - anionic fluorinated surfactant - 1 wt.%.

A receptor element was prepared. Methyl hydroxy propyl cellulose (10 wt. % solution in water) was coated onto a subbed 75 µm polyethylene terephthalate film from an aqueous solution to form a receptor element comprising a polyethylene terephthalate support base and an image receiving layer of 10 µm thickness. The sub comprised a 1 wt.% methanol solution of "Elvamide 8063" (c) - coated using a 6 thou. (152 µm) Meyer bar.

The resulting receptor element was passed through a typical commercial ink-jet printer ( Hewlett Packard HP550 at 300dpi) connected to a personal computer and the liquid containing the chemical agent was applied in a preprogrammed manner to form the desired image. The receptor element was then placed on a glass plate, with the coated layer facing uppermost. The receptor element was covered with a screen mesh of mesh count 62 threads per cm. Then a bead of a typical (but unsensitized) polyvinylalcohol/polyvinyl acetate screen emulsion - "2000" (b) - was placed on the upper side of the mesh and drawn over the receptor element by means of a squeegee so that a thin layer of emulsion was forced through the mesh. After 1 minute, the polyethylene terephthalate support base was removed from the mesh. The resulting screen was left to dry and then washed out using cold running water, until the portion of the assembly of higher solubility was washed away to waste.

The stencil was then placed in a standard screen printing machine and prints of an acceptable quality were obtained using standard solvent-based screen printing inks.

### EXAMPLE 2

A liquid containing a first chemical agent was prepared according to the formula:
water - 50 wt.%; and
"Quilon C" (b) - pentahydroxy(tetradecanoate)dichromium, 50 wt.%.
"Quilon C" is itself a 25% solution in acetone/isopropyl alcohol.

Polyvinylpyrrolidone (10 wt.% solution in water) was coated onto a 75 µm polyethylene terephthalate film from an aqueous solution to form a receptor element comprising a polyethylene terephthalate support base and an image receiving layer of 10 µm thickness.

The resulting receptor element was passed through a typical commercial ink-jet printer (Hewlett Packard HP550 at 300dpi) connected to a personal computer and the liquid containing the chemical agent was applied in a preprogrammed manner to form the desired image. The receptor element was then placed on a glass plate, with the coated layer facing uppermost. The receptor element was covered with a screen mesh of mesh count 62 threads per cm. Then a bead of a typical (but unsensitized) polyvinylalcohol/polyvinyl acetate screen emulsion - "2000" (c) - was placed on the upper side of the mesh and drawn over the receptor element by means of a squeegee so that a thin layer of emulsion was forced through the mesh. The polyethylene terephthalate support base was removed from the mesh. The resulting screen was left to dry thoroughly using a hot air fan and then washed out using cold running water, until the portion of the assembly of higher solubility was washed away to waste.

The stencil was then placed in a standard screen printing machine and prints of an acceptable quality were obtained using standard solvent-based screen printing inks.

### EXAMPLE 3

The procedure of Example 1 above was repeated exactly to produce a screen stencil.

This stencil was then treated with a 10 wt. % aqueous solution of potassium carbonate, which was applied by brush so as to cover the entire stencil area, then finally allowed to dry. This produced a toughened stencil, which was placed in a standard screen printing machine and prints of an acceptable quality were obtained using standard solvent-based screen printing inks.

### EXAMPLE 4

The procedure of Example 1 above was repeated exactly to produce a screen stencil.

This stencil was then treated with a 2 wt.% solution of 35 wt.% hydrochloric acid, which was applied by brush so as to cover the entire stencil area. This treatment disrupted the screen stencil and allowed the resulting residue to be washed away to waste using a cold water spray, giving a reclaimed screen with no observable stain present.

### EXAMPLE 5

A liquid containing a chemical agent was prepared according to the formula:
water - 87 wt.%;
potassium tetraborate - 10 wt.%;
borax - 2 wt.%; and
"Fluorad FC-93" (a) (1wt. % aqueous solution) - anionic fluorinated surfactant - 1 wt.%.

Polyvinyl alcohol - "Gohsenol GH-20" (d) (10 wt.% solution in water) of hydrolysis 88% and degree of polymerisation 2000, was coated onto a unsubbed 75 µm polyethylene terephthalate film from an aqueous solution to form a receptor element comprising a polyethylene terephthalate support base and an image receiving layer of 10 microns thickness.

The resulting receptor element was passed through a typical commercial ink-jet printer (Hewlett Packard HP550 at 300dpi) connected to a personal computer and the liquid containing the chemical agent was applied in a preprogrammed manner to form the desired image.

The receptor element was dried, then placed on a glass plate, with the coated layer facing uppermost. The receptor element was covered with a screen mesh of mesh count 62 threads per cm. Then a bead of a typical (but unsensitized) polyvinylalcohol/polyvinyl acetate screen emulsion - "2000" (c) - was placed on the mesh and drawn over the receptor element by means of a squeegee so that a thin layer of emulsion was forced through the mesh. The screen was dried by hot air fan until the polyethylene terephthalate support base could be peeled cleanly from the mesh. The screen was left to dry and then washed out using cold running water, until the portion of the assembly of higher solubility was washed away to waste.

The stencil was then placed in a standard screen printing machine and prints of an acceptable quality were obtained using standard solvent-based screen printing inks.

### EXAMPLE 6

A 50:50 wt.% blend of polyvinyl alcohol - "Gohsenol GH-20" (d) and polyvinyl acetate was coated onto an unsubbed 75 µm microns polyethylene terephthalate film from an aqueous solution to form a receptor element comprising a polyethylene terephthalate support base and an image-receiving layer of 10 µm thickness.

The resulting receptor element was passed through a typical commercial ink-jet printer (Hewlett Packard HP550 at 300 dpi) connected to a personal computer and liquid containing a chemical agent was applied according to the formula:
water - 50 wt.%; and
"Quilon C" (b) - pentahydroxy(tetradecanoate)dichromium, 50 wt.%. "Quilon C" is itself a 25% solution in acetone/isopropyl alcohol.

The receptor element was then treated in exactly the same manner as in Example 5 above.

The stencil was then placed in a standard screen printing machine and prints of an acceptable quality were obtained using standard solvent-based screen printing inks.

### EXAMPLE 7

The procedure of Example 5 above was repeated exactly to produce a screen stencil.

This stencil was then treated with a 10 wt.% solution of potassium carbonate which was applied by brush so as to cover the entire stencil area, then finally allowed to dry. This produced a toughened stencil, which was placed in a standard screen printing machine and prints of an acceptable quality were obtained using standard solvent-based screen printing inks.

### EXAMPLE 8

The procedure of Example 5 above was repeated exactly to produce a screen stencil.

This stencil was then treated with a 5 wt.% solution of glacial acetic acid, which was applied by brush so as to cover the entire stencil area. This treatment disrupted the screen stencil and allowed the resulting residue to be washed away to waste using a cold water spray, giving a reclaimed screen with no observable stain present.

## Claims

1. A method of producing a screen-printing stencil having open areas and blocked areas for respectively passage and blocking of a printing medium, the method comprising:
providing a receptor element comprising an image-receiving layer capable of receiving a first chemical agent in areas corresponding to the blocked areas of the stencil to be produced;
applying the first chemical agent to the image-receiving layer of the receptor element in the said corresponding areas;
applying a second, stencil-forming chemical agent to a screen printing screen,
bringing the image-receiving layer of the receptor element into contact with the stencil-forming agent, to allow the first and second chemical agents to react to produce on the screen a stencil-forming layer having areas of lower solubility corresponding to the said blocked areas and areas of higher solubility in areas corresponding to the open stencil areas;
removing any remaining unreacted part of the receptor element; and
washing away the second chemical agent in the higher solubility areas, thereby to produce the screen-printing stencil.

2. A method according to claim 1, wherein the first chemical agent is produced *in situ* by reaction between two or more precursor materials, separately applied to the image-receiving layer, prior to contact with the stencil forming agent, at least one of which is applied in the said areas corresponding to the blocked areas of the stencil to be produced.

3. A method according to claim 1 or 2, wherein the image-receiving layer of the receptor element reacts with the first chemical agent to produce lower solubility areas corresponding to the said blocked areas and excess of the first chemical agent remains in said areas to react with the second chemical agent upon contact between the image-receiving layer and the stencil-forming agent, whereby the respective lower solubility areas of the image-receiving layer and of the stencil-forming layer combine with one another and, after the higher solubility areas are washed away, remain to form the blocked areas of the screen-printing stencil.

4. A method according to claims 1 or 2, wherein the image-receiving layer comprises one or more of the following polymers: methyl hydroxy propyl cellulose, carboxymethyl cellulose, polyvinylpyrrolidone and polyacrylic acids.

5. A method according to any of claims 1 to 3, wherein the image-receiving layer comprises paper.

6. A method according to claim 4, wherein the polymer(s) is/are present in the image-receiving layer in a total amount of 5 to 100 wt % of the image-receiving layer.

7. A method according to claim 6, wherein the image-receiving layer contains one or more of: fillers, binders and plasticisers.

8. A method according to claim 3, wherein the image-receiving layer comprises one or more of the following polymers:
polyvinylalcohol and its derivatives;
gelatin and its derivatives;
carboxylated polymers capable of becoming water soluble on addition of alkali;
water-soluble cellulose derivatives;
sulphonated polymers;
polyacrylamides;
epoxy resins; and
amino resins.

9. A method according to claim 8, wherein the image-receiving layer comprises, as a said carboxylated polymer, carboxylated acrylic polymer, an ethylene-acrylic acid copolymer or a styrene-acrylic acid polymer.

10. A method according to claim 8, wherein the image-receiving. layer comprises, as a water-soluble cellulose derivative, starch or hydroxypropyl cellulose.

11. A method according to claim 8, wherein the image-receiving layer comprises, as an amino resin, a urea-formaldehyde resin or a melamine-formaldehyde resin.

12. A method according to claim 8, wherein the image-receiving layer comprises polyvinyl alcohol with a degree of hydrolysis of from 20 to 99.9 mole % and/or a degree of polymerisation of from 100 to 3500.

13. A method according to any preceding claim, wherein the receptor element includes a support base.

14. A method according to claim 13, wherein the support base is from 10 to 200µm in thickness.

15. A method according to claim 14, wherein the support base comprises polyethylene terephthalate, polyethylene, polycarbonate, polyvinyl chloride, polystyrene or a coated paper.

16. A method according to claim 14 or 15, wherein the image-receiving layer has a thickness of from 0.1 to 50 µm.

17. A method according to any of claims 1 to 12, wherein the receptor element has no support base and the image-receiving layer has a thickness of from 6 to 250 µm.

18. A method according to any preceding claim, wherein the second chemical agent comprises one or more of the following polymers:
polyvinylalcohol and its derivatives;
gelatin and its derivatives;
carboxylated polymers capable of becoming water soluble on addition of alkali;
water-soluble cellulose derivatives;
sulphonated polymers;
polyacrylamides;
epoxy resins; and
amino resins.

19. A method according to claim 18, wherein the second chemical agent comprises, as a said carboxylated polymer, a carboxylated acrylic polymer, an ethylene-acrylic acid copolymer or a styrene-acrylic acid copolymer.

20. A method according to claim 18, wherein the second chemical agent comprises, as a water-soluble cellulose derivative, starch or hydroxypropyl cellulose.

21. A method according to claim 18, wherein the second chemical agent comprises, as an amino resin, a urea-formaldehyde resin or a melamine formaldehyde resin.

22. A method according to any preceding claim, wherein the active component(s) of the first chemical agent comprises one or more of:
boron salts;
boric acid;
aldehydes;
isocyanates;
isocyanate derivatives;
carbodiimides;
carbodiimide derivatives;
transition metal compounds;
transition metal complexes;
aziridine;
aziridine derivatives;
amines;
multifunctional silane compounds;
N-methylol compounds; and
active vinyl compounds.

23. A method according to claim 22, wherein the active component(s) of the first chemical agent comprises one or more Group I or Group II metal borates.

24. A method according to claim 22, wherein the active component(s) of the first chemical agent comprises formaldehyde.

25. A method according to claim 22, wherein the active component(s) of the first chemical agent comprises a dialdehyde.

26. A method according to claim 25, wherein the dialdehyde is glyoxal or glutaraldehyde.

27. A method according to claim 26, wherein the dialdehyde is activated by treatment with mineral acid.

28. A method according to claim 22, wherein the active component(s) of the first chemical agent comprises toluenediisocyanate.

29. A method according to claim 22, wherein the active component(s) of the first chemical agent comprises 1,3-dicyclohexylcarbodiimide.

30. A method according to claim 22, wherein the active component(s) of the first chemical agent comprises pentahydroxy (tetradecanoate) dichromium or a derivative thereof.

31. A method according to claim 22, wherein the active component(s) of the first chemical agent comprises silicon tetraacetate.

32. A method according to claim 22, wherein the active component(s) of the first chemical agent comprises dimethylolurea or methyloldimethylhydantoin.

33. A method according to claim 22, wherein the active component(s) of the first chemical agent comprises 1, 3, 5-triacryloyl-hexahydro-*s*-triazine.

34. A method according to any preceding claim, wherein the active component(s) of the first chemical agent constitutes from 0.5 to 100 wt.% of the first chemical agent.

35. A method according to claim 2, wherein the first chemical agent precursor applied in the areas corresponding to the blocked areas of the stencil to be produced comprises a reactive dialdehyde and a further first chemical agent precursor is a dilute acid.

36. A method according to claim 35, wherein the reactive dialdehyde is water-soluble.

37. A method according to claim 36, wherein the dialdehyde is glyoxal or glutaraldehyde.

38. A method according to any of claims 35 to 37, wherein the dilute acid is an acid which lowers the pH to 4 or less when mixed with the dialdehyde.

39. A method according to claim 38, wherein the acid is hydrochloric acid or citric acid.

40. A method according to any preceding claim, wherein the first chemical agent is applied dropwise to the receptor element.

41. A method according to claim 40, wherein the dropwise application is by an ink-jet printer or an ink-jet plotter.

42. A method according to claim 41, wherein the ink-jet printer or plotter has more than one ejection head.

43. A method according to any of claims 1 to 39, wherein the first chemical agent is supplied to the receptor element by a hand-held delivery device.

44. A method according to any preceding claim, wherein the stencil is further toughened by a post-treatment using further chemicals, actinic radiation or heat.

45. A method according to claim 44, wherein the further chemicals for further chemical toughening are resident in the image-receiving layer and/or in the stencil-forming agent.

46. A method according to claim 44, wherein the further chemicals are applied image-wise.

47. A method according to any of claims 44 to 46, wherein the further chemicals include an aqueous base.

48. A method according to claim 47, wherein the base is potassium carbonate.

49. A method according to any preceding claim, including a further, reclaim step.

50. A method according to claim 49, wherein the first chemical agent comprises a borate and the reclaim is carried out at a pH of 4 or less.

51. A method according to any preceding claim, wherein the second chemical agent is applied to the screen printing screen from one side thereof after the receptor element has been applied to the other side thereof with its image-receiving layer in contact with the screen, whereby the image-receiving layer is brought onto contact with the second chemical agent.

52. A method according to any of claims 1 to 50, wherein the second chemical agent is applied to the screen printing screen and the receptor element is subsequently brought into contact with the screen to bring the image-receiving layer thereof into contact with the second chemical agent.

53. A method according to any preceding claim, wherein any support base present is removed before washing away the second chemical agent in the higher solubility areas.

54. A method according to any of claims 1 to 52, wherein any support base present is removed by the washing away of the second chemical agent in the higher solubility areas.

55. A method of screen printing comprising the steps of:
providing a screen printing stencil produced by a method according to any of claims 1 to 54,
placing the screen printing stencil in contact with a substrate, and
passing a printing medium through the open areas of the stencil to produce printing on the substrate in areas corresponding to the open areas of the stencil.

56. A pre-filled cartridge for a dropwise application device, the cartridge containing a chemical agent which comprises one or more of the following as an active component in an amount of from 0.5 to 100 wt % of the chemical agent:
boron salts;
boric acid;
aldehydes;
isocyanates;
isocyanate derivatives;
carbodiimides;
carbodiimide derivatives;
transition metal compounds;
transition metal complexes;
aziridine;
aziridine derivatives;
amines;
multifunctional silane compounds;
N-methylol compounds; and
active vinyl compounds.

57. A pre-filled cartridge according to claim 56, wherein the active component of the chemical agent comprises one or more Group I or Group II metal borate.

58. A pre-filled cartridge according to claim 56, wherein the active component of the chemical agent comprises formaldehyde.

59. A pre-filled cartridge according to claim 56, wherein the active component of the chemical agent comprises a dialdehyde.

60. A pre-filled cartridge according to claim 59, wherein the dialdehyde is glyoxal or glutaraldehyde.

61. A pre-filled cartridge according to claim 60, wherein the dialdehyde is activated by treatment with mineral acid.

62. A pre-filled cartridge according to claim 56, wherein the active component of the chemical agent comprises toluenediisocyanate.

63. A pre-filled cartridge according to claim 56, wherein the active component of the chemical agent comprises 1,3-dicyclohexylcarbodiimide.

64. A pre-filled cartridge according to claim 56, wherein the active component of the chemical agent comprises pentahydroxy (tetradecanoate) dichromium or a derivative thereof.

65. A pre-filled cartridge according to claim 56, wherein the active component of the chemical agent comprises silicon tetraacetate.

66. A pre-filled cartridge according to claim 56, wherein the active component of the chemical agent comprises dimethylolurea or methyloldimethylhydantoin.

67. A pre-filled cartridge according to claim 56, wherein the active component of the chemical agent comprises 1, 3, 5-triacryloyl-hexahydro-*s*-triazine.

68. A cartridge for an ink-jet printer or plotter, according to any of claims 56 to 67.

## Patentansprüche

1. Verfahren zur Herstellung einer Siebdruckschablone mit offenen Bereichen und blockierten Bereichen für die Passage bzw. das Blockieren eines Druckmediums, wobei das Verfahren Folgendes umfasst:
Vorsehen eines Aufnahmeelementes, das eine bildaufnehmende Schicht umfasst, die zum Aufnehmen eines ersten chemischen Mittels in Bereichen fähig ist, die den blockierten Bereichen der herzustellenden Schablone entsprechen;
Aufbringen des ersten chemischen Mittels auf die bildaufnehmende Schicht des Aufnahmeelementes in den genannten entsprechenden Bereichen;
Aufbringen eines zweiten schablonenbildenden chemischen Mittels auf ein Siebdrucksieb,
Inkontaktbringen der bildaufnehmenden Schicht des Aufnahmeelementes mit dem schablonenbildenden Mittel, um den ersten und zweiten chemischen Mitteln zu ermöglichen, zur Herstellung auf dem Sieb einer schablonenbildenden Schicht mit Bereichen von geringerer Löslichkeit, die den genannten blockierten Bereichen entsprechen und Bereichen von höherer Löslichkeit in Bereichen, die den offenen Schablonenbereichen entsprechen, zu reagieren;
Entfernen von jeglichem zurückbleibendem, nicht zur Reaktion gebrachtem Teil des Aufnahmeelementes; und
Auswaschen des zweiten chemischen Mittels in den Bereichen von höherer Löslichkeit, um dadurch die Siebdruckschablone herzustellen.

2. Verfahren nach Anspruch 1, worin das erste chemische Mittel *in situ* durch Reaktion zwischen zwei oder mehr Präkursor-Materialien hergestellt wird, die vor dem Kontakt mit dem schablonenbildenden Mittel getrennt auf die bildaufnehmende Schicht aufgebracht werden, wobei mindestens eine von diesen in den genannten Bereichen aufgebracht wird, die den blockierten Bereichen der herzustellenden Schablone entsprechen.

3. Verfahren nach Anspruch 1 oder 2, worin die bildaufnehmende Schicht des Aufnahmeelementes mit dem ersten chemischen Mittel reagiert, um Bereiche von geringerer Löslichkeit herzustellen, die den genannten blockierten Bereichen entsprechen und ein Überschuss des ersten chemischen Mittels in genannten Bereichen zurückbleibt, um mit dem zweiten chemischen Mittel nach Kontakt zwischen der bildaufnehmenden Schicht und der schablonenbildenden Schicht zu reagieren, wobei die entsprechenden Bereiche von geringerer Löslichkeit der bildaufnehmenden Schicht und der schablonenbildenden Schicht sich miteinander vereinigen und, nachdem die Bereiche von höherer Löslichkeit ausgewaschen wurden, zur Bildung der blockierten Bereiche der Siebdruckschablone zurückbleiben.

4. Verfahren nach Anspruch 1 oder 2, worin die bildaufnehmende Schicht ein Polymer oder mehrere der folgenden Polymere umfasst: Methylhydroxypropylcellulose, Carboxymethylcellulose, Polyvinylpyrrolidon und Polyacrylsäuren.

5. Verfahren nach einem der Ansprüche 1 bis 3, worin die bildaufnehmende Schicht Papier umfasst.

6. Verfahren nach Anspruch 4, worin das/die Polymer(e) in der bildaufnehmenden Schicht in einer Gesamtmenge von 5 bis 100 Gew.-% der bildaufnehmenden Schicht vorliegt/vorliegen.

7. Verfahren nach Anspruch 6, worin die bildaufnehmende Schicht eines oder mehreres von Folgendem enthält: Füllstoffe, Bindemittel und Weichmacher.

8. Verfahren nach Anspruch 3, worin die bildaufnehmende Schicht ein Polymer oder mehrere der folgenden Polymere umfasst:
Polyvinylalkohol und seine Derivate;
Gelatine und ihre Derivate;
carboxylierte Polymere, die nach Zufügen von Alkali dazu fähig sind, wasserlöslich zu werden;
wasserlösliche Cellulose-Derivate;
sulfonierte Polymere;
Polyacrylamide;
Epoxidharze und
Aminoharze.

9. Verfahren nach Anspruch 8, worin die bildaufnehmende Schicht, als ein genanntes carboxyliertes Polymer, carboxyliertes Acrylpolymer, ein Ethylen-Acrylsäure-Copolymer oder ein Styren-Acrylsäure-Polymer umfasst.

10. Verfahren nach Anspruch 8, worin die bildaufnehmende Schicht, als ein wasserlösliches Cellulose-Derivat, Stärke oder Hydroxylpropylcellulose umfasst.

11. Verfahren nach Anspruch 8, worin die bildaufnehmende Schicht, als ein Aminoharz, ein Harnstoff-Formaldehyd-Harz oder ein Melamin-Formaldehyd-Harz umfasst.

12. Verfahren nach Anspruch 8, worin die bildaufnehmende Schicht Polyvinylalkohol mit einem Hydrolysegrad von 20 bis 99,9 Mol-% und/oder einen Polymerisationsgrad von 100 bis 3500 umfasst.

13. Verfahren nach einem der vorangehenden Ansprüche, worin das Aufnahmeelement eine Trägerbasis einschließt.

14. Verfahren nach Anspruch 13, worin die Trägerbasis von 10 bis 200 µm dick ist.

15. Verfahren nach Anspruch 14, worin die Trägerbasis Polyethylenterephthalat, Polyethylen, Polycarbonat, Polyvinylchlorid, Polystyren oder ein gestrichenes Papier umfasst.

16. Verfahren nach Anspruch 14 oder 15, worin die bildaufnehmende Schicht eine Dicke von 0,1 bis 50 µm aufweist.

17. Verfahren nach einem der Ansprüche 1 bis 12, worin das Aufnahmeelement keine Trägerbasis besitzt und die bildaufnehmende Schicht eine Dicke von 6 bis 250 µm aufweist.

18. Verfahren nach einem der vorangehenden Ansprüche, worin das zweite chemische Mittel ein Polymer oder mehrere der folgenden Polymere umfasst:
Polyvinylalkohol und seine Derivate;
Gelatine und seine Derivate;
carboxylierte Polymere, die nach Zufügen von Alkali dazu fähig sind, wasserlöslich zu werden;
wasserlösliche Cellulosederivate;
sulfonierte Polymere;
Polyacrylamide;
Epoxidharze und
Aminoharze.

19. Verfahren nach Anspruch 18, worin das zweite chemische Mittel, als ein genanntes carboxyliertes Polymer, ein carboxyliertes Acrylpolymer, ein Ethylen-Acrylsäure-Copolymer oder ein Styren-Acrylsäure-Copolymer umfasst.

20. Verfahren nach Anspruch 18, worin das zweite chemische Mittel, als ein wasserlösliches Cellulosederivat, Stärke oder Hydroxypropylcellulose umfasst.

21. Verfahren nach Anspruch 18, worin das zweite chemische Mittel, als ein Aminoharz, ein Harnstoff-Formaldehyd-Harz oder ein Melamin-Formaldehyd-Harz umfasst.

22. Verfahren nach einem der vorangehenden Ansprüche, worin die aktive(n) Komponente(n) des ersten chemischen Mittels eines oder mehreres des Folgenden umfasst/umfassen:
Borsalze;
Borsäure;
Aldehyde;
Isocyanate;
Isocyanat-Derivate;
Carbodiimide;
Carbodiimid-Derivate;
Übergangsmetallverbindungen;
Übergangsmetallkomplexe;
Aziridin;
Aziridin-Derivate;
Amine;
multifunktionale Silanverbindungen;
N-Methylol-Verbindungen und
aktive Vinylverbindungen.

23. Verfahren nach Anspruch 22, worin die aktive(n) Komponente(n) des ersten chemischen Mittels ein Metallborat oder mehrere Metallborate der Gruppe I oder Gruppe II umfasst/umfassen.

24. Verfahren nach Anspruch 22, worin die aktive(n) Komponente(n) des ersten chemischen Mittels Formaldehyd umfasst/umfassen.

25. Verfahren nach Anspruch 22, worin die aktive(n) Komponente(n) des ersten chemischen Mittels einen Dialdehyd umfasst/umfassen.

26. Verfahren nach Anspruch 25, worin der Dialdehyd Glyoxal oder Glutaraldehyd ist.

27. Verfahren nach Anspruch 26, worin der Dialdehyd durch Behandlung mit Mineralsäure aktiviert wird.

28. Verfahren nach Anspruch 22, worin die aktive(n) Komponente(n) des ersten chemischen Mittels Toluendiisocyanat umfasst/umfassen.

29. Verfahren nach Anspruch 22, worin die aktive(n) Komponente(n) des ersten chemischen Mittels 1,3-Dicyclohexylcarbodiimid umfasst/umfassen.

30. Verfahren nach Anspruch 22, worin die aktive(n) Komponente(n) des ersten chemischen Mittels Pentahydroxy(tetradecanoat)dichrom oder ein Derivat davon umfasst/umfassen.

31. Verfahren nach Anspruch 22, worin die aktive(n) Komponente(n) des ersten chemischen Mittels Siliciumtetraacetat umfasst/umfassen.

32. Verfahren nach Anspruch 22, worin die aktive(n) Komponente(n) des ersten chemischen Mittels Dimethylolharnstoff oder Methyloldimethylhydantoin umfasst/umfassen.

33. Verfahren nach Anspruch 22, worin die aktive(n) Komponente(n) des ersten chemischen Mittels 1,3,5-Triacryloyl-hexahydro-s-triazin umfasst/umfassen.

34. Verfahren nach einem der vorangehenden Ansprüche, worin die aktive(n) Komponente(n) des ersten chemischen Mittels von 0,5 bis 100 Gew.-% des ersten chemischen Mittels ausmacht.

35. Verfahren nach Anspruch 2, worin der Präkursor des ersten chemischen Mittels in den Bereichen aufgebracht wird, die den blockierten Bereichen der herzustellenden Schablone entsprechen, einen reaktiven Dialdehyd umfasst und ein weiterer Präkursor des ersten chemischen Mittels eine verdünnte Säure ist.

36. Verfahren nach Anspruch 35, worin der reaktive Dialdehyd wasserlöslich ist.

37. Verfahren nach Anspruch 36, worin der Dialdehyd Glyoxal oder Glutaraldehyd ist.

38. Verfahren nach einem der Ansprüche 35 bis 37, worin die verdünnte Säure eine Säure ist, die den pH auf 4 oder niedriger senkt, wenn sie mit dem Dialdehyd vermischt wird.

39. Verfahren nach Anspruch 38, worin die Säure Salzsäure oder Citronensäure ist.

40. Verfahren nach einem der vorangehenden Ansprüche, worin das erste chemische Mittel tropfenweise auf das Aufnahmeelement aufgebacht wird.

41. Verfahren nach Anspruch 40, worin das tropfenweise Aufbringen durch einen Tintenstrahldrucker oder einen Tintenstrahlplotter vorgenommen wird.

42. Verfahren nach Anspruch 41, worin der Tintenstrahldrucker oder -plotter mehr als einen Strahldüsenkopf hat.

43. Verfahren nach einem der Ansprüche 1 bis 39, worin das erste chemische Mittel durch eine Handabgabevorrichtung an das Aufnahmeelement geliefert wird.

44. Verfahren nach einem der vorangehenden Ansprüche, worin die Schablone ferner durch eine Nachbehandlung unter Verwendung weiterer Chemikalien, aktinischer Strahlung oder Hitze gehärtet wird.

45. Verfahren nach Anspruch 44, worin die weiteren Chemikalien zur weiteren chemischen Härtung in der bildaufnehmenden Schicht und/oder in dem schablonenbildenden Mittel resident sind.

46. Verfahren nach Anspruch 44, worin die weiteren Chemikalien bildweise aufgebracht werden.

47. Verfahren nach einem der Ansprüche 44 bis 46, worin die weiteren Chemikalien eine wässrige Base einschließen.

48. Verfahren nach Anspruch 47, worin die Base Kaliumcarbonat ist.

49. Verfahren nach einem der vorangehenden Ansprüche, das einen weiteren Regenerierungsschritt einschließt.

50. Verfahren nach Anspruch 49, worin das erste chemische Mittel ein Borat umfasst und die Regenerierung bei einem pH von 4 oder weniger ausgeführt wird.

51. Verfahren nach einem der vorangehenden Ansprüche, worin das zweite chemische Mittel auf das Siebdrucksieb von einer Seite davon aufgebracht wird, nachdem das Aufnahmeelement auf der anderen Seite davon aufgebracht worden ist, wobei sich seine bildaufnehmende Schicht in Kontakt mit dem Sieb befindet, wobei die bildaufnehmende Schicht mit dem zweiten chemischen Mittel in Kontakt gebracht wird.

52. Verfahren nach einem der Ansprüche 1 bis 50, worin das zweite chemische Mittel auf das Siebdrucksieb aufgebracht wird und das Aufnahmeelement anschließend in Kontakt mit dem Sieb gebracht wird, um die bildaufnehmende Schicht davon in Kontakt mit dem zweiten chemischen Mittel zu bringen.

53. Verfahren nach einem der vorangehenden Ansprüche, worin jede vorliegende Trägerbasis vor dem Auswaschen des zweiten chemischen Mittels in den Bereichen von höherer Löslichkeit entfernt wird.

54. Verfahren nach einem der Ansprüche 1 bis 52, worin jedwede vorliegende Trägerbasis durch Auswaschen des zweiten chemischen Mittels in den Bereichen von höherer Löslichkeit entfernt wird.

55. Verfahren zum Siebdrucken, das die folgenden Schritte umfasst:
Vorsehen einer Siebdruckschablone, die durch ein Verfahren nach einem der Ansprüche 1 bis 54 hergestellt wird,
Inkontaktbringen der Siebdruckschablone mit einem Substrat und
Durchleiten eines Drackmediums durch die offenen Bereiche der Schablone, um Bedrucken auf dem Substrat in den Bereichen herbeizuführen, die den offenen Bereichen der Schablone entsprechen.

56. Eine vorbefüllte Kartusche für eine Vorrichtung zum tropfenweisen Aufbringen, wobei die Kartusche ein chemisches Mittel enthält, das eines oder mehreres des Folgenden als eine aktive Komponente in einer Menge von 0,5 bis 100 Gew.-% des chemischen Mittels umfasst:
Borsalze;
Borsäure;
Aldehyde;
Isocyanate;
Isocyanat-Derivate;
Carbodiimide;
Carbodiimid-Derivate;
Übergangsmetallverbindungen;
Übergangsmetallkomplexe;
Aziridin;
Aziridin-Derivate;
Amine;
multifunktionale Silanverbindungen;
N-Methylol-Verbindungen und
aktive Vinylverbindungen.

57. Vorbefüllte Kartusche nach Anspruch 56, worin die aktive Komponente des chemischen Mittels ein Metallborat oder mehrere Metallborate der Gruppe I oder Gruppe II umfasst.

58. Vorbefüllte Kartusche nach Anspruch 56, worin die aktive Komponente des chemischen Mittels Formaldehyd umfasst.

59. Vorbefüllte Kartusche nach Anspruch 56, worin die aktive Komponente des chemischen Mittels einen Dialdehyd umfasst.

60. Vorbefüllte Kartusche nach Anspruch 59, worin der Dialdehyd Glyoxal oder Glutaraldehyd ist.

61. Vorbefüllte Kartusche nach Anspruch 60, worin der Dialdehyd durch Behandlung mit Mineralsäure aktiviert wird.

62. Vorbefüllte Kartusche nach Anspruch 56, worin die aktive Komponente des chemischen Mittels Toluendiisocyanat umfasst.

63. Vorbefüllte Kartusche nach Anspruch 56, worin die aktive Komponente des chemischen Mittels 1,3-Dicyclohexylcarbodiimid umfasst.

64. Vorbefüllte Kartusche nach Anspruch 56, worin die aktive Komponente des chemischen Mittels Pentahydroxy(tetradecanoat)dichrom oder ein Derivat davon umfasst.

65. Vorbefüllte Kartusche nach Anspruch 56, worin die aktive Komponente des chemischen Mittels Siliciumtetraacetat umfasst.

66. Vorbefüllte Kartusche nach Anspruch 56, worin die aktive Komponente des chemischen Mittels Dimethylolharnstoff oder Methyloldimethylhydantoin umfasst.

67. Vorbefüllte Kartusche nach Anspruch 56, worin die aktive Komponente des chemischen Mittels l,3,5-Triacryloyl-hexahydro-s-triazin umfasst.

68. Kartusche für einen Tintenstrahldrucker oder -plotter nach einem der Ansprüche 56 bis 67.

## Revendications

1. Méthode de production d'un pochoir pour sérigraphie ayant des zones ouvertes et des zones bloquées pour, respectivement, le passage et le blocage d'un milieu d'impression, la méthode comprenant :
la fourniture d'un élément récepteur comprenant une couche de réception d'image susceptible de recevoir un premier agent chimique dans des zones correspondant aux zones bloquées du pochoir à produire ;
l'application du premier agent chimique à la couche de réception d'image de l'élément récepteur dans lesdites zones correspondantes;
l'application d'un deuxième agent chimique formateur de pochoir à un écran de sérigraphie ;
la mise en contact de la couche de réception d'image de l'élément récepteur avec l'agent formateur de pochoir, pour permettre au premier et au deuxième agents chimiques de réagir pour produire sur l'écran une couche formatrice de pochoir ayant des zones de solubilité inférieure correspondant auxdites zones bloquées et des zones de solubilité supérieure dans des zones correspondant aux zones de pochoir ouvertes ;
l'élimination de toute partie non réagie restante de l'élément récepteur ; et
l'élimination par lavage du deuxième agent chimique dans les zones de solubilité supérieure, produisant ainsi le pochoir pour sérigraphie.

2. Méthode selon la revendication 1, dans laquelle le premier agent chimique est produit *in situ* par une réaction entre deux ou plusieurs matériaux précurseurs, appliqués séparément à la couche de réception d'image, préalablement au contact avec l'agent formateur de pochoir, dont au moins un est appliqué dans lesdites zones correspondant aux zones bloquées du pochoir à produire.

3. Méthode selon la revendication 1 ou 2, dans laquelle la couche de réception d'image de l'élément récepteur réagit avec le premier agent chimique pour produire des zones de solubilité inférieure correspondant auxdites zones bloquées et l'excès en premier agent chimique reste dans lesdites zones pour réagir avec le deuxième agent chimique lors du contact entre la couche de réception d'image et l'agent formateur de pochoir, ce par quoi les zones de solubilité inférieure respectives de la couche de réception d'image et de la couche formatrice de pochoir s'associent l'une à l'autre et, après l'élimination par lavage des zones de solubilité supérieure, restent pour former les zones bloquées du pochoir de sérigraphie.

4. Méthode selon la revendication 1 ou 2, dans laquelle la couche de réception d'image comprend un ou plusieurs parmi les polymères suivants : la méthylhydroxypropyl cellulose, la carboxyméthyl cellulose, la polyvinylpyrrolidone et les acides polyacryliques.

5. Méthode selon l'une quelconque des revendications 1 à 3, dans laquelle la couche de réception d'image comprend du papier.

6. Méthode selon la revendication 4, dans laquelle le ou les polymère(s) est(sont) présent(s) dans la couche de réception d'image en une quantité totale allant de 5 à 100% en poids de la couche de réception d'image.

7. Méthode selon la revendication 6, dans laquelle la couche de réception d'image contient un ou plusieurs parmi : les charges, les liants et les plastifiants.

8. Méthode selon la revendication 3, dans laquelle la couche de réception d'image comprend un ou plusieurs parmi les polymères suivants :
l'alcool polyvinylique et ses dérivés ;
la gélatine et ses dérivés ;
les polymères carboxylés susceptibles de devenir hydrosolubles lors de l'addition de base ;
les dérivés de cellulose hydrosolubles ;
les polymères sulfonés ;
les polyacrylamides ;
les résines époxy ; et
les résines aminées.

9. Méthode selon la revendication 8, dans laquelle la couche de réception d'image comprend, comme dit polymère carboxylé, un polymère acrylique carboxylé, un copolymère d'éthylène-acide acrylique ou un polymère de styrène-acide acrylique.

10. Méthode selon la revendication 8, dans laquelle la couche de réception d'image comprend, comme dérivé de cellulose hydrosoluble, de l'amidon ou de l'hydroxypropyl cellulose.

11. Méthode selon la revendication 8, dans laquelle la couche de réception d'image comprend, comme résine aminée, une résine d'urée-formol ou une résine de mélamine-formol.

12. Méthode selon la revendication 8, dans laquelle la couche de réception d'image comprend de l'alcool polyvinylique ayant un degré d'hydrolyse allant de 20 à 99,9% molaire et/ou un degré de polymérisation allant de 100 à 3 500.

13. Méthode selon l'une quelconque des revendications précédentes, dans laquelle l'élément récepteur comporté une base de support.

14. Méthode selon la revendication 13, dans laquelle l'épaisseur de la base de support va de 10 à 200 µm.

15. Méthode selon la revendication 14, dans laquelle la base de support comprend du polytéréphtalate d'éthylène, du polyéthylène, du polycarbonate, du chlorure polyvinylique, du polystyrène ou un papier revêtu.

16. Méthode selon la revendication 14 ou 15, dans laquelle l'épaisseur de la couche de réception d'image va de 0,1 à 50 µm.

17. Méthode selon l'une quelconque des revendications 1 à 12, dans laquelle l'élément récepteur n'a pas de base de support et l'épaisseur de la couche de réception d'image va de 6 à 250 µm.

18. Méthode selon l'une quelconque des revendications précédentes, dans laquelle le deuxième agent chimique comprend un ou plusieurs parmi les polymères suivants :
l'alcool polyvinylique et ses dérivés ;
la gélatine et ses dérivés ;
les polymères carboxylés susceptibles de devenir hydrosolubles lors de l'addition de base ;
les dérivés de cellulose hydrosolubles ;
les polymères sulfonés ;
les polyacrylamides ;
les résines époxy ; et
les résines aminées.

19. Méthode selon la revendication 18, dans laquelle le deuxième agent chimique comprend, comme dit polymère carboxylé, un polymère acrylique carboxylé, un copolymère d'éthylène-acide acrylique ou un copolymère de styrène-acide acrylique.

20. Méthode selon la revendication 18, dans laquelle le deuxième agent chimique comprend, comme dérivé de cellulose hydrosoluble, de l'amidon ou de l'hydroxypropyl cellulose.

21. Méthode selon la revendication 18, dans laquelle le deuxième agent chimique comprend, comme résine aminée, une résine d'urée-formol ou une résine de mélamine-formol.

22. Méthode selon l'une quelconque des revendications précédentes, dans laquelle le ou les composant(s) actif(s) du premier agent chimique comprend(comprennent) un ou plusieurs parmi :
les sels de bore ;
l'acide borique ;
les aldéhydes ;
les isocyanates ;
les dérivés d'isocyanate ;
les carbodiimides ;
les dérivés de carbodiimide ;
les composés de métaux dé transition ;
les complexes de métaux de transition ;
I'aziridine ;
les dérivés d'aziridine ;
les amines ;
les composés de silane multifonctionnels ;
les composés de N-méthylol ; et
les composés vinyliques actifs.

23. Méthode selon la revendication 22, dans laquelle le ou les composant(s) actif(s) du premier agent chimique comprend(comprennent) un ou plusieurs borates de métaux du Groupe I ou du Groupe II.

24. Méthode selon la revendication 22, dans laquelle le ou les composant(s) actif(s) du premier agent chimique comprend(comprennent) du formaldéhyde.

25. Méthode selon la revendication 22, dans laquelle le ou les composant(s) actif(s) du premier agent chimique comprend(comprennent) un dialdéhyde.

26. Méthode selon la revendication 25, dans laquelle le dialdéhyde est le glyoxal ou le glutaraldéhyde.

27. Méthode selon la revendication 26, dans laquelle le dialdéhyde est activé par un traitement par de l'acide minéral.

28. Méthode selon la revendication 22, dans laquelle le ou les composant(s) actif(s) du premier agent chimique comprend(comprennent) du toluènediisocyanate.

29. Méthode selon la revendication 22, dans laquelle le ou les composant(s) actif(s) du premier agent chimique comprend(comprennent) du 1,3-dicyclohexylcarbodiimide.

30. Méthode selon la revendication 22, dans laquelle le ou les composant(s) actif(s) du premier agent chimique comprend(comprennent) du pentahydroxy(tétradécanoate)dichromium ou un dérivé de celui-ci.

31. Méthode selon la revendication 22, dans laquelle le ou les composant(s) actif(s) du premier agent chimique comprend(comprennent) du tétraacétate de silicium.

32. Méthode selon la revendication 22, dans laquelle le ou les composant(s) aetif(s) du premier agent chimique comprend(comprennent) de la diméthylolurée ou de la méthyloldiméthylhydantoïne.

33. Méthode selon la revendication 22, dans laquelle le ou les composant(s) actif(s) du premier agent chimique comprend(comprennent) de la 1,3,5-triacryloylhexahydro-s-triazine.

34. Méthode selon l'une quelconque des revendications précédentes, dans laquelle le ou les composant(s) actif(s) du premier agent chimique constitue(nt) de 0,5 à 100% en poids du premier agent chimique.

35. Méthode selon la revendication 2, dans laquelle le précurseur du premier agent chimique appliqué dans les zones correspondant aux zones bloquées du pochoir à produire comprend un dialdéhyde réactif et un précurseur supplémentaire du premier agent chimique est un acide dilué.

36. Méthode selon la revendication 35, dans laquelle le dialdéhyde réactif est hydrosoluble.

37. Méthode selon la revendication 36, dans laquelle le dialdéhyde est le glyoxal ou le glutaraldéhyde.

38. Méthode selon l'une quelconque des revendications 35 à 37, dans laquelle l'acide dilué est un acide qui abaisse le pH jusqu'à 4 ou moins, lors de son mélange avec le dialdéhyde.

39. Méthode selon la revendication 38, dans laquelle l'acide est l'acide chlorhydrique ou l'acide citrique.

40. Méthode selon l'une quelconque des revendications précédentes, dans laquelle le premier agent chimique est appliqué goutte-à-goutte à l'élément récepteur.

41. Méthode selon la revendication 40, dans laquelle l'application goutte-à-goutte est réalisée par une imprimante à jet d'encre ou un traceur à jet d'encre.

42. Méthode selon la revendication 41, dans laquelle l'imprimante ou le traceur à jet d'encre possède plus d'une tête d'éjection.

43. Méthode selon l'une quelconque des revendications 1 à 39, dans laquelle le premier agent chimique est fourni à l'élément récepteur par un dispositif d'alimentation portatif.

44. Méthode selon l'une quelconque des revendications précédentes, dans laquelle le pochoir est durci davantage par un post-traitement à l'aide de produits chimiques supplémentaires, de rayonnement actinique ou de chaleur.

45. Méthode selon la revendication 44, dans laquelle les produits chimiques supplémentaires pour un durcissement chimique supplémentaire résident dans la couche de réception d'image et/ou dans l'agent formateur de pochoir.

46. Méthode selon la revendication 44, dans laquelle les produits chimiques supplémentaires sont appliqués image par image.

47. Méthode selon l'une quelconque des revendications 44 à 46, dans laquelle les produits chimiques supplémentaires comportent une base aqueuse.

48. Méthode selon la revendication 47, dans laquelle la base est le carbonate de potassium.

49. Méthode selon l'une quelconque des revendications précédentes, comportant une étape supplémentaire de récupération.

50. Méthode selon la revendication 49, dans laquelle le premier agent chimique comprend un borate et la récupération est réalisée à un pH de 4 ou moins.

51. Méthode selon l'une quelconque des revendications précédentes, dans laquelle le deuxième agent chimique est appliqué à l'écran de sérigraphie depuis l'un des côtés de celui-ci après l'application de l'élément récepteur à l'autre côté de celui-ci, sa couche de réception d'image étant en contact avec l'écran, ce par quoi la couche de réception d'image est mise en contact avec le deuxième agent chimique.

52. Méthode selon l'une quelconque des revendications 1 à 50, dans laquelle le deuxième agent chimique est appliqué à l'écran de sérigraphie et l'élément récepteur est ultérieurement mis en contact avec l'écran pour mettre en contact la couche de réception d'image de celui-ci avec le deuxième agent chimique.

53. Méthode selon l'une quelconque des revendications précédentes, dans laquelle toute base de support présente est éliminée avant l'élimination par lavage du deuxième agent chimique dans les zones de solubilité supérieure.

54. Méthode selon l'une quelconque des revendications 1 à 52, dans laquelle toute base de support présente est éliminée par l'élimination par lavage du deuxième agent chimique dans les zones de solubilité supérieure.

55. Méthode de sérigraphie comprenant les étapes de :
fourniture d'un pochoir pour sérigraphie produit par une méthode selon l'une quelconque des revendications 1 à 54,
positionnement du pochoir pour sérigraphie en contact avec un substrat, et
passage d'un milieu d'impression à travers les zones ouvertes du pochoir pour produire une impression sur le substrat dans des zones correspondant aux zones ouvertes du pochoir.

56. Cartouche préalablement remplie pour un dispositif d'application goutte-à-goutte, la cartouche contenant un agent chimique comprenant un ou plusieurs parmi les suivants comme composant actif en une quantité allant de 0,5 à 100% en poids de l'agent chimique :
les sels de bore ;
l'acide borique ;
les aldéhydes ;
les isocyanates ;
les dérivés d'isocyanate ;
les carbodiimides ;
les dérivés de carbodiimide ;
les composés de métaux de transition ;
les complexes de métaux de transition ;
l'aziridine ;
les dérivés d'aziridine ;
les amines ;
les composés de silane multifonctionnels ;
les composés de N-méthylol ; et
les composés vinyliques actifs.

57. Cartouche préalablement remplie selon la revendication 56, dans laquelle le composant actif de l'agent chimique comprend un ou plusieurs borates de métaux du Groupe I ou du Groupe II.

58. Cartouche préalablement remplie selon la revendication 56, dans laquelle le composant actif de l'agent chimique comprend du formaldéhyde.

59. Cartouche préalablement remplie selon la revendication 56, dans laquelle le composant actif de l'agent chimique comprend un dialdéhyde.

60. Cartouche préalablement remplie selon la revendication 59, dans laquelle le dialdéhyde est le glyoxal ou le glutaraldéhyde.

61. Cartouche préalablement remplie selon la revendication 60, dans laquelle le dialdéhyde est activé par un traitement par un acide minéral.

62. Cartouche préalablement remplie selon la revendication 56, dans laquelle le composant actif de l'agent chimique comprend du toluènediisocyanate.

63. Cartouche préalablement remplie selon la revendication 56, dans laquelle le composant actif de l'agent chimique comprend du 1,3-dicyclohexylcarbodiimide.

64. Cartouche préalablement remplie selon la revendication 56, dans laquelle le composant actif de l'agent chimique comprend du pentahydroxy(tétradécanoate)dichromium ou un dérivé de celui-ci.

65. Cartouche préalablement remplie selon la revendication 56, dans laquelle le composant actif de l'agent chimique comprend du tétraacétate de silicium.

66. Cartouche préalablement remplie selon la revendication 56, dans laquelle le composant actif de l'agent chimique comprend de la diméthylolurée ou de la méthyloldiméthylhydantoïne.

67. Cartouche préalablement remplie selon la revendication 56, dans laquelle le composant actif de l'agent chimique comprend de la 1,3,5-triacryloylhexahydro-*s*-triazine.

68. Cartouche pour une imprimante ou un traceur à jet d'encre, selon l'une quelconque des revendications 56 à 67.
